

## UNITED STATES PATENT OFFICE

JOHN C. EMHARDT, OF NEWBURGH, NEW YORK, ASSIGNOR TO E. I. DU PONT DE NEMOURS & COMPANY, OF WILMINGTON, DELAWARE, A CORPORATION OF DELAWARE

## NITROCELLULOSE COMPOSITION

No Drawing.

Application filed September 21, 1926. Serial No. 136,896.

This invention relates to cellulose nitrate compositions containing semi-drying vegetable oil, e. g. blown castor, cottonseed or rapeseed oil as a softener, and, more particularly, it relates to such compositions having such a degree of non-stickiness that the compositions will be, even when freshly spread on the backing of artificial leather, adaptable to high-production processes of manufacture. 5 When softeners of the type indicated are used in the ordinary manner they give a coating so sticky that the goods cannot be handled with desired rapidity in the machines, i. e. cannot be folded, rolled, and so on substantially immediately after coating. The present 10 composition provides a proper coating for the purposes indicated. It is the major object of the invention to provide such a composition. 15 According to the present invention there is used in the composition a suitable quantity of mineral oil to overcome and eliminate the stickiness imparted by the vegetable oil. The "mineral oil" is preferably a non-volatile, 20 oily paraffin or naphthene hydrocarbon. The coating resulting from the composition, after evaporating the volatile solvents from a coating composition having the composition of the invention as its base, will not be tacky even 25 when hot. This permits the coated goods, e. g. leather substitute, to come in contact with itself or the machine immediately, without objectionable results. 30

It is to be noted that the vegetable oils mentioned are non-solvent softeners for cellulose nitrate, i. e. while softeners they are not solvents. It is the particular present desire to provide compositions which shall be free from solvent softeners, e. g. tricresyl phosphate, 35 dibutyl phthalate, etc., that is, will have their softener content composed of non-solvent softeners. The use of the mineral oil, meets this condition since it is a non-solvent softener and can satisfactorily serve alone as a 40 stickiness reducer. In this aspect the present compositions are to be clearly distinguished from compositions that might be devised, containing a solvent softener as its primary softener, a non-solvent softener, and mineral oil. 45 When the mineral oil is used with the vege-

table oils as specified no difficulty is experienced from precipitation of the pyroxylin.

Compositions in accordance with the invention may be as follows (parts by weight):—

| Pigmented      |            | 55        |
|----------------|------------|-----------|
|                | Range      | Preferred |
| Nitrocellulose | 16         | 16        |
| Pigment (dry)  | 10         | 10        |
| Vegetable oil  | 33.32-32.3 | 32.98     |
| Mineral oil    | .68-1.6    | 1.02      |

  

| Clear          |            | 65        |
|----------------|------------|-----------|
|                | Range      | Preferred |
| Nitrocellulose | 16         | 16        |
| Vegetable oil  | 15.68-15.2 | 15.52     |
| Mineral oil    | .32-.8     | .48       |

As will be understood by those skilled in the art of making artificial leather, the mixtures covered by the above examples are dissolved in an amount of a suitable solvent (e. g., benzol 3, ethyl acetate 2), to give a desired "jelly", 114 parts by weight of the said solvent giving substantially a 16 ounce jelly, but other jellies may, of course, be used; and the resulting solution is then applied to a fabric and allowed to evaporate in the regular way. The particular difference, in manufacturing 75 the present goods, from manufacturing prior goods, will be found in the increased speed with which the operation can be carried on, due to the elimination of stickiness.

The compositions may be used for under coats or top coats as experience and desire dictate. The pigment may be any desired one, as bone black, and the vegetable oil is, as before noted, desirably blown castor, blown cottonseed, or blown rapeseed. In the "pigmented" formula, it will be seen that the mineral oil is from 2% substantially to, but not including, 5% of the total oil, while in the "clear" formula the mineral oil varies from 2% to 5% of the total oil. Both formulas can vary 85 in blown oil content from 1 to 3 parts of oil to 1 part of nitrocellulose. In the "pigmented" formula the pigment content can vary 90 from 1 to 2½ parts of pigment to 1 part of nitrocellulose. Ordinarily, of course, the 95

pigmented composition will be used for under coats and the clear composition for the top coat.

While the use of the composition in the making of leather substitute has been more particularly referred to, it will be understood that it may be otherwise used. While more particular reference to blown oils has been made, it will be understood that the invention is applicable to compositions containing raw oils which are non-solvent softeners for cellulose nitrate.

I claim:

- 15 1. A homogeneous nitrocellulose composition free from solvent softeners and containing nitrocellulose, a blown semi-drying vegetable oil, and non-volatile mineral oil in an amount substantially between 2 and 5% of the total mineral and vegetable oil content.
- 20 2. A homogeneous nitrocellulose composition free from solvent softeners and containing nitrocellulose, a blown vegetable oil of the group, castor, cottonseed and rapeseed, and non-volatile mineral oil in an amount substantially between 2 and 5% of the total mineral and vegetable oil content.
- 25 3. A homogeneous pyroxylin coating composition, free from solvent softeners and containing, as a softener for the coating, a blown semi-drying vegetable oil in an amount that, if used alone, would impart stickiness to the coating, and non-volatile mineral oil as a thickness preventive.
- 30 4. A homogeneous nitrocellulose composition containing nitrocellulose, and, as a softener for the nitrocellulose a non-solvent-softener mixture comprising a blown vegetable oil of the group, castor, cottonseed and rapeseed, and non-volatile mineral oil in an amount substantially between 2 and 5% of the total mineral and vegetable oil content.
- 35 5. A homogeneous pyroxylin coating composition, free from solvent softeners and containing, as a softener for the coating, a blown semi-drying vegetable oil, and a non-volatile mineral oil as a stickiness preventive.

In testimony whereof I affix my signature.

JOHN C. EMHARDT.